

# UNITED STATES PATENT OFFICE.

DANIEL MANSON SUTHERLAND, OF ASHGROVE, ENGLAND.

## VARNISH FOR APPLYING TO FABRICS OF AEROPLANES.

1,320,290.

Specification of Letters Patent. Patented Oct. 28, 1919.

No Drawing.

Application filed August 2, 1918. Serial No. 247,905.

To all whom it may concern:

Be it known that I, DANIEL MANSON SUTHERLAND, a subject of the King of Great Britain, residing at Ashgrove, Sunbury Common, in the county of Middlesex, England, have invented new and useful Improvements in Varnishes or Dopes More Especially Intended for Applying to the Fabrics of Aeroplanes and other Aerial Machines, of which the following is a specification.

In varnishes or dopes containing acetyl cellulose as at present used on the fabrics covering the wings and other parts of aeroplanes, or other aerial machines, triphenyl phosphate has been employed in as high a proportion as 15 parts of triphenyl phosphate to 85 parts of acetyl cellulose, triphenyl phosphate being a scarce and expensive commodity.

The object of the present invention is to produce a suitable varnish or dope without the employment of triphenyl phosphate by the use of ingredients readily obtainable in this country and less costly.

According to this invention I have discovered that in place of triphenyl phosphate, boric acid can be advantageously employed; this is added in suitable proportions preferably to benzol, and together they form one of the ingredients of an acetyl cellulose varnish or dope, the benzol thus preferably displacing the alcohol or the like hitherto in use, so that in a varnish or dope according to this invention boric acid displaces triphenyl phosphate, or its equivalent while the alcohol, or the like, is preferably displaced by benzol, and a larger proportion of the benzol is used than has been possible hitherto; such combination of benzol with boric acid, I term borated benzol.

A dope or varnish so produced possesses excellent fire resisting qualities, the drying of the varnish is advantageously retarded, its viscosity diminished so that more highly concentrated solutions of the acetyl cellulose in the varnish can be used and the said varnish does not readily chill and turn white.

I have found the following examples yield a good serviceable and durable var-

nish or dope but the invention is not limited to the said examples or to the proportions stated given therein which will vary according to the consistency, viscosity and other particular properties required.

Example 1. (A thin varnish).

|                                             | Parts by weight. |
|---------------------------------------------|------------------|
| Acetyl cellulose                            | 6                |
| Acetone or other equivalent solvent         | 44               |
| Benzol (preferably 90%)                     | 24               |
| Borated benzol (boric acid 10%, benzol 90%) | 24 65            |
| Benzyl alcohol                              | 2                |
|                                             | 100              |

Example 2. (A medium varnish).

|                                            | Parts by weight. |
|--------------------------------------------|------------------|
| Acetyl cellulose                           | 12               |
| Acetone or other equivalent solvent        | 36               |
| Benzol (preferably 90%)                    | 24 75            |
| Borated benzol—boric acid 10%, benzol 90%) | 25               |
| Benzyl alcohol                             | 3                |
|                                            | 100 80           |

In some instances benzol may advantageously be replaced by benzene used in or about the same proportions as indicated in the examples for benzol.

Although I have described the use of boric acid and benzol, termed borated benzol, in the foregoing examples, for the production of acetyl cellulose varnishes as more especially applicable for varnishing fabrics for aero machines, it must be understood that the invention is not limited thereto but that the borated benzol may also be used in the production of other varnishes or dopes for example, in varnishes or dopes in which nitro-cellulose or celluloid replaces the acetyl cellulose or its equivalent such for example as what are known as "non-flam" films.

What I claim is:

1. A cellulosic varnish comprising borated benzol as an essential ingredient thereof.

2. A cellulosic varnish comprising cellulosic material, a solvent therefor, benzol, borated benzol and benzyl alcohol.

3. A cellulose varnish comprising acetyl cellulose, acetone, benzol, borated benzol and benzyl alcohol.

In testimony whereof I have signed my

name to this specification in the presence of two subscribing witnesses.

DANIEL MANSON SUTHERLAND.

Witnesses:

G. E. TYSON,  
L. WALTER.